

April 7, 1936.

A. D. SLACK

2,036,440

NONHALATION PHOTOGRAPHIC FILM

Filed Feb. 18, 1931

Fig.1.



Fig.2.



Fig.3.



Inventor

Alfred D. Slack,

By

Newton M. Perkins

Attorney

## UNITED STATES PATENT OFFICE

2,036,440

## NONHALATION PHOTOGRAPHIC FILM

Alfred D. Slack, Rochester, N. Y., assignor to  
Eastman Kodak Company, Rochester, N. Y., a  
corporation of New York

Application February 18, 1931, Serial No. 516,629

11 Claims. (CL. 95—9)

The following described invention relates to photographic film and particularly to the prevention or reduction of halation in the photographic image.

Although my invention is in no way limited in its application to motion picture film alone, its characteristics are such that its use in this field results in a decided improvement in picture quality and, when used in conjunction with sound recording on film, results in improved tone reproduction.

Halation and its troubles are well known to those versed in the photographic art, but its prevention or reduction involves a problem which has presented many difficulties.

Motion picture film, when developed after exposure, is customarily processed in machines through which it is passed continuously. When some medium has been incorporated in or on the film as a means of eliminating or reducing halation, it is accordingly undesirable that this non-halation layer shall become gummy and stick to the gears or foul the developing baths. It is also deleterious if this backing shall be removed in coherent films or scales. Such large pieces or particles are apt to become attached to the sensitized emulsion face of the film and thus interfere with the normal action of the processing baths.

In order to avoid certain of such difficulties a non-halation layer should either be completely soluble or destroyed in one or any of the photographic baths, or be removed in such sized particles as to obviate any danger of interference with normal processing. In those instances where a dyestuff has been utilized as the non-halation medium, it is furthermore undesirable to use a dyestuff which will be soluble in any of the photographic baths. Such a coloring material would be released into the baths and tend to stain either the emulsion or the base of succeeding film as it passes through the processing machine.

If dyestuffs are applied directly to the material comprising the film support, the dyes utilized may or may not be soluble or diluted with solvents which penetrate the support, at least sufficiently to give the dyes firm adherence. If these dyes be water soluble, or soluble in the normal baths a staining of the emulsion or base may occur as related above. However, if dyes which are not soluble in water or the photographic baths or destroyed in the regular processing baths are used, they are usually difficult

of complete removal, although they may be removed by special bleach baths.

If a completely water soluble insulating layer or carrier for the non-halation layer or dye be used, it has the disadvantage of becoming soft under moist atmospheric conditions.

I overcame all of the above difficulties by utilizing as an insulating layer a layer of material which is insoluble in water and therefore does not tend to become soft or sticky under moist or damp atmospheric conditions. However, the material is completely soluble in an alkaline bath, such as that which comprises the normal photographic developing solution. While this material may be permeable to or somewhat absorptive of water, it is not attacked by those solvents ordinarily utilized for the usual cellulosic support.

If a film support be coated with a layer of such material and there is then applied a dyestuff insoluble in the photographic baths, from a solvent which does not penetrate through the said layer into the film base, the dye will remain as a very thin coating directly over and on the backing layer. This layer thus effectually prevents the dye from reaching the material of the film support.

When such a film is processed, the developer permeates the outer dye layer and attacks the insulating layer of casein which is completely dissolved in the alkaline developer and will thus necessarily be removed from the film support, carrying the overcoat dye layer with it, leaving the film base clear and stainless. Moreover, as the dyestuff is insoluble both in the water and any of the normal processing baths, it will neither attack nor stain either the film base or the emulsion, but will float off in minute particles. Those materials which I have found most suitable are such proteins as casein, gliadin, zein, glutenin, and albumen. These may be used alone or mixed together as desired.

If a carrier layer which is not so impervious to water as the above mentioned materials is found suitable for the purpose desired, other substances may be used. Such materials are dextrose, gum arabic, or other similar water soluble substances.

However, I have found casein to be particularly desirable. The type of casein which I employ is soluble in glacial acetic acid and may be diluted to any consistency with ethyl alcohol or other alcohols. If an acetic acid-casein solution is not desirable, an alkaline solution of casein may be used. The casein is not water soluble, though

a layer of it may be somewhat permeable to water. It is, however, completely soluble in an alkaline bath, although its solubility in the baths may be decreased if desired by the addition of 5 formalin, hexa-methylene-tetramine, certain metal salts or the like.

In order to incorporate all of the above mentioned desirable features in a non-halation backing, a layer of the casein is coated upon the film base. To this coated layer there may be applied a suitable dye or combination of dyes, which are not soluble either in water or the developing baths, but are soluble either in a material which is a solvent of the film support or at 10 least penetrates the support. While a mixture of complementary dyes is often utilized in compounding an anti-halation backing with fairly good success, I have found, that, for optimum 15 quality, a black dye is most desirable. As a panchromatized emulsion (which is sensitive throughout the visible spectrum) is now frequently used, a backing material which is about 20 equally absorptive to light throughout the visible spectrum is ideal. In such a case a blue 25 black dye may be perfectly satisfactory as the sensitizing dye incorporated in the panchromatic emulsion so effectually absorbs light in the blue portion of the spectrum, that the resulting effectual anti-halation qualities closely approach 30 those of a pure jet black.

The ideal dyestuff to use would be one whose absorption most nearly approaches that of carbon.

Typical solvents for such dyestuffs are amyl 35 acetate, ethyl acetate, carbon tetrachloride, ethyl alcohol, acetone, or ethylene dichloride etc. If it be desired that the dyes shall penetrate more or less into the backing layer, without, however, 40 saturating it to such an extent as to stain the support, this may be accomplished by including with the dye solution a higher alcohol or other material which will prolong the drying time and thus increase the degree of dye penetration into 45 the layer. Water may also effectually be used to accomplish this end. If 5% of water be used, a partial penetration can be obtained, and with a larger percentage any degree of penetration 50 can be procured to the extent even that the film base itself may be stained.

If it be found that the resultant backing is too 55 brittle for normal use, flexibilizers such as glycerin, rubber latex, triacetin, or other materials may be added. These will be completely removed from the base at the time of processing.

Typical formulæ for the insulating layer are 60 as follows:

|                     |            |
|---------------------|------------|
| Casein              | 100 grams  |
| Glacial acetic acid | 250 c. c.  |
| Ethyl alcohol       | 3250 c. c. |
| or                  |            |
| Casein              | 100 grams  |
| Ammonia             | 100 c. c.  |
| Water               | 1050 c. c. |
| Ethyl alcohol       | 2350 c. c. |

Typical dye solutions which have been found useful are the following:

|                    |            |
|--------------------|------------|
| Oil red O          | 50 grams   |
| Oil blue B         | 50 grams   |
| Ethyl acetate      | 3500 c. c. |
| or                 |            |
| Spirit nigrosine R | 50 grams   |
| Ethyl alcohol      | 1900 c. c. |

Water may be added to the last formula, the amount added being dependent on the extent to which it is desired that the dyestuff shall penetrate the insulating layer. I have found 100 5 c. c. to be satisfactory.

In order to make the invention clearer, reference is made to the accompanying drawing in which:

Fig. 1 is a section of a film constituting a preferred embodiment of my invention.

Fig. 2 is a section of another embodiment, and

Fig. 3 is a section of still a third embodiment.

The support 2 is of a composition such as is customary for this purpose, usually comprising cellulose nitrate, acetate, ether or other derivative. It has on one surface a photographically sensitive layer 1. The water permeable layer 15 is designated as 3 and the dye layer as 4.

If the dye is caused to penetrate the permeable layer as in Fig. 2 it may cease to be distinguishable as a separate layer and there will result a unitary layer 5 which is heavily dyed at and near its outer surface and of graded dye intensity decreasing with the depth of the layer.

The support need not be a single unitary layer 25 but may comprise several permanent layers. The main support may carry a secondary surface layer for anti-static or non-curling purposes. Such secondary layer would be of a composition different from the main support layer, but permanently adherent thereto under all conditions and usage. It may for instance be of a cellulose derivative different from the main support or it may be of hardened gelatine, hardened casein, an insoluble or hardened gum or other 35 material. In such a case a governing factor will be the affinity of the insulating layer or the solvents carrying it for this secondary support layer. Such an embodiment is illustrated in Fig. 3 wherein the main support layer 2 carries on one surface a sensitive layer 1 and has permanently adherent to the other surface a secondary support layer 6 over which is the insulating layer 3 which protects the layer 6 from the dye layer 4 or the solvent used in applying the 40 dye. When the film is processed, the layers 3 and 4 are removed leaving a clear and unstained 45 support.

It is to be understood that I contemplate as included within my invention all such modifications and equivalents as fall within the scope of the appended claims.

What I claim as new and desire to be secured by Letters Patent of the United States is:

1. A photographic film comprising a light 55 transmitting, flexible support, a photographically sensitive layer on one surface thereof and a halation reducing backing on the other surface thereof, said backing comprising a carrier and a dye, predominantly at the outer surface thereof, the carrier being soluble in photographic baths and the dye having a tendency to stain permanently the surface of the support, the carrier constituting a layer insulating said surface from the dye.

2. A photographic film comprising a light 70 transmitting, flexible support, a photographically sensitive layer on one surface thereof and a halation reducing backing on the other surface thereof, said backing comprising a water permeable layer and, directly applied to the surface thereof, a dye having a tendency to stain permanently the surface of the support, the water permeable layer insulating the surface from the dye.

3. A photographic film comprising a light transmitting, flexible support, a photographically sensitive layer on one surface thereof and a halation reducing backing on the other surface thereof, said backing comprising a water permeable layer carrying directly applied to the surface thereof a dye which is soluble in a solvent that attacks the material of the support but not of the backing layer.

10 4. A photographic film comprising a light transmitting, flexible support, a sensitive gelatine emulsion on one surface thereof and a halation reducing backing on the other surface thereof, said backing comprising a layer of material which is removable in the photographic baths and carrying at its outer surface a dye which is insoluble in water but soluble in a solvent which attacks the material of the support but not of the backing and which does not tend 15 to stain gelatine.

15 5. A photographic film comprising a support of a cellulosic composition, a sensitive emulsion on one surface thereof, and a non-halation backing on the other surface thereof, said backing comprising a layer of material permeable to but insoluble in water and soluble in ordinary photographic baths and carrying directly applied to the surface thereof a dye which is water insoluble, but soluble in a solvent that attacks the 20 material of the support but not of the backing layer.

25 6. A photographic film comprising a light-transmitting, flexible support, a sensitive emulsion on one surface thereof, and a halation-reducing backing on the other surface thereof, said backing comprising a colloidal layer of a protein which is permeable to but insoluble in water and soluble in an alkali solution and carrying directly on its outer surface a dye which 30 is insoluble in water, but soluble in a solvent which attacks the material of the support but not of the backing.

35 7. A photographic film comprising a light-transmitting, flexible support, a sensitive emulsion on one surface thereof and a halation-reducing backing on the other surface thereof, said backing comprising a colloidal layer of a casein which is permeable to but insoluble in water and soluble in 40

an alkali solution and carrying applied directly to the outer surface thereof a dye which is insoluble in water but soluble in a solvent which attacks the material of the support but not of the backing.

5 8. A photographic film comprising a support of cellulosic composition, a sensitive emulsion on one surface thereof, and a non-halation backing on the other surface thereof, said backing comprising a layer soluble in water or the regular 10 developing baths, and carrying applied directly to the outer surface thereof a dye which is insoluble in water and the regular developing baths, but soluble in a solvent which may attack the material of the support, but not of the backing 15 layer.

9. The method of rendering free from halation a photographic film having a light-transmitting support susceptible to certain solvents that comprises applying to said support a layer 20 that is permeable to water, removable in ordinary photographic baths, and unaffected by said certain solvents, applying to said layer a dye in solution in one of said solvents whereby said layer prevents the dye solution from reaching 25 and staining said support whereby there may be used for anti-halation purposes dyes that otherwise would be unavailable because of their tendency to stain the support.

10. The method of reducing halation in a 30 photographic film having a light-transmitting support susceptible to certain solvents that comprises applying to said support a layer of a protein that is permeable to but not soluble in water, but which is soluble in ordinary photographic baths, applying to said layer a dye in 35 solution in a solvent that does not affect said protein but which does attack the support.

11. The method of reducing halation in a photographic film having a light-transmitting 40 cellulosic support susceptible to certain solvents that comprises applying to said support a layer of casein which is soluble in an alkali solution and then applying to said casein layer a solution of dye in a readily evaporative solvent that 45 does not affect the casein but which is capable of attacking the material of the support.

ALFRED D. SLACK.